

July 18, 1950

W. D. NICOLL

2,515,889

PROCESS FOR PRODUCING ARTIFICIAL FILAMENTS

Filed Jan. 28, 1949

2 Sheets-Sheet 1



*Fig. 1.*



*Fig. 2.*

William D. Nicoll INVENTOR.

BY

Charles F. Daley  
ATTORNEY

July 18, 1950

W. D. NICOLL

2,515,889

PROCESS FOR PRODUCING ARTIFICIAL FILAMENTS

Filed Jan. 28, 1949

2 Sheets-Sheet 2



*Fig. 3.*



*Fig. 4.*

William D. Nicoll INVENTOR.

BY  
Charles F. Daley  
ATTORNEY

## UNITED STATES PATENT OFFICE

2,515,889

PROCESS FOR PRODUCING ARTIFICIAL  
FILAMENTS

William D. Nicoll, Wilmington, Del., assignor to  
E. I. du Pont de Nemours & Company, Wil-  
mington, Del., a corporation of Delaware

Continuation of abandoned application Serial No.  
477,720, March 2, 1943. This application Jan-  
uary 28, 1949, Serial No. 73,323

19 Claims. (Cl. 18—54)

1

This invention relates to the production of crimped, wool-like filaments and fibers comprising regenerated cellulose and a protein.

This application is a continuation of my co-pending application Serial No. 477,720, filed March 2, 1943, now abandoned.

Many attempts have been made, heretofore, to produce a wool-like fiber or filament comprised of regenerated cellulose and a protein. Such fibers have great utility in producing mixed rayon-wool yarns and fabrics which can be dyed to substantially uniform color with wool dyes.

Crimped, regenerated cellulose-protein filaments and fibers, as produced prior to this invention, have lacked one essential character of wool, namely, the ability to retain a substantial crimp after being subjected to a material stretch.

My co-pending application Serial No. 465,414, filed November 13, 1942, covers a process for the production of unique, permanently crimped wool-like regenerated cellulose filaments and fibers. It has now been found that similar unique, permanently crimped regenerated cellulose-protein filaments and fibers can be produced in a similar manner.

It is therefore an object of this invention to produce new and unique, crimped regenerated cellulose-protein filaments and fibers which will retain a substantial crimp after being subjected to a material stretch, and which filaments and fibers have a high wet and dry tenacity.

It is still another object of this invention to produce regenerated cellulose-protein filaments and fibers which will crimp instantaneously upon being suspended, free from tension, in an aqueous bath having a shrinking action on said filaments.

It is another object of the invention to produce new and unique crimped regenerated cellulose-protein filaments and fibers in which the crimp, after being removed mechanically, such as by stretching, combing or the like, will be substantially completely restored by suspending the same, free from tension, in an aqueous liquid having a shrinking action on said filaments.

Other objects of the invention will appear hereinafter.

Similar to my copending application above referred to, viscose-sulfuric acid-salt systems in which the minimum gel swelling factor of the regenerated cellulose filaments obtainable therefrom is less than 6.5 will hereinafter be referred to as "balanced viscose-sulfuric acid-salt spinning bath systems."

The gel swelling factor of regenerated cellu-

2

lose filaments is determined in the following manner:

A viscose of known composition is extruded through a spinneret into a sulfuric acid coagulating bath of known composition. The coagulated filaments, after leaving the bath, are wound in a single layer on to a bobbin with a helical wind of narrow pitch in such a manner that successive windings are very closely spaced. When the bobbin contains 2 to 6 grams of wet gel yarn, the bobbin is removed and rotated on a chuck to centrifuge off the bath carried with the filaments on to the bobbin. The acid-wet gel yarn is then cut from the bobbin and weighed. The whole operation should be carried out within four minutes. The acid-wet gel yarn is washed and then dried to remove all the water therefrom and the dry yarn reweighed. The ratio of the weight of acid-wet gel yarn to the weight of the dry yarn is termed its "gel swelling factor."

It is possible for this gel swelling factor to range from about 3 to about 12, depending upon the composition of the viscose and of the coagulating bath. For a given viscose composition, a high concentration of sulfuric acid in the coagulating bath will result in the production of a regenerated cellulose having a high gel swelling factor. If the acidity is gradually decreased (with the composition of the viscose and coagulating bath otherwise remaining the same), the gel swelling factor falls to a minimum and then rises again with a further decrease in the acidity. The gel swelling factor at the minimum will be termed the "minimum gel swelling factor," and the acidity at this point will be termed the "minimum gel swelling factor acidity."

The above objects can be accomplished, in general, by preparing a viscose composition containing 5% to 100% protein, based on the weight of the cellulose in the viscose, and spinning filaments from said viscose composition in a coagulating and regenerating bath while observing the following highly critical combination of conditions: Spinning filaments in a balanced viscose-sulfuric acid-salt spinning bath system in which the spinning bath contains zinc sulfate and the sulfuric acid content of the bath is between 60% and 90% of the minimum gel swelling factor acidity; imposing on said filaments, during the spinning thereof, a tension of at least 0.5 gram per denier and a stretch of at least 40%; and, after substantially complete regeneration of said filaments, relaxing the same completely free of all tension in a liquid which will swell the same. [By "stretch of at least 40%" is meant

a stretch (as measured between the point where the spun filaments are first converged in the bath, and collecting device) of at least 40%, based on its unstretched length.] For practical purposes, it is generally desirable that the coagulating bath have a temperature of between 40° C. and 75° C. and preferably that the zinc sulfate content of the bath be from 0.1% to 3%.

The methods and means by which the present invention may be carried out will be apparent by reference to the following detailed description when taken in connection with the accompanying illustration, in which:

Figure 1 is a diagrammatic view, with parts shown in perspective, of one form of apparatus suitable for use in accordance with the present invention;

Figure 2 is a similar diagrammatic perspective view, with parts shown in perspective, of another modified form of apparatus for use in accordance with the present invention;

Figure 3 is a diagrammatic view of still another modified form of apparatus suitable for use in carrying out the present invention;

Figure 4 is a typical gel swelling factor curve.

Referring to Figure 1, reference numeral 11 designates a conduit line for a viscose-protein filament forming composition which is connected to any suitable source of supply. The conduit 11 is connected in the usual manner to a candle filter 12, and the candle filter 12 is connected to a spinneret 14 by means of a "goose-neck" 13. The viscose solution is extruded through the spinneret 14 to form filaments 15. The bundle of filaments is passed about the convergence guide 16 and thence about roller guides 17 and take-off guide 18. From guide 18 the yarn is passed about a feed wheel 19 from which the yarn is fed through two vertically spaced sleeve guides 21 and 23. If desired, a liquid may be passed through the two sleeve guides by means of a nozzle 24. The liquid will continuously force the yarn through the two sleeve guides. A rotatable cutter knife 25 may be positioned to rotate between the two sleeve guides 21 and 23, thereby cutting the yarn into small staple lengths. The cutter knife is mounted on a shaft 27 and is adapted to be rotated by means of a driven belt. The staple fibers 28 drop into a relaxing fluid 29 where they will be completely free from tension and will be substantially instantaneously crimped along the length thereof.

Referring to Figure 2 of the drawings, the yarn 15, after passing from the feed wheel 19, is led directly to a relaxing bath contained in container 21, while completely freeing the yarn from tension. A short length of yarn is permitted to accumulate in the bottom of the container 21. As soon as the yarn strikes the bath, it will be substantially instantaneously crimped as shown at 23. The yarn is continuously removed from the container 21 by passing the same over rotatable guide 25 and wound on to a bobbin 31 which may be driven by surface drive roller 33. The yarn may be traversed on the bobbin in the conventional manner by means of a traverse guide 35. In passing between the bath and the bobbin, the yarn is dried by means of a forced draft drier 27. Just prior to winding the yarn on the bobbin 31, it may be slightly tensioned by means of pinch tensioning device 29.

Referring to Figure 3 of the drawings, the yarn 15, composed of freshly spun filaments, is passed from the spinneret 14 about fixed convergence guide 16, then through a long bath tank 20 to

a take-off guide 18. The yarn is then passed to draw-off rollers 30 and 32 which are of sufficient size to provide a surface area of sufficient extent to eliminate any material slippage of the yarn thereon. The yarn is then passed from draw-off roller 32 about guide roller 43, and then about stretching rollers 45 and 47. The yarn passes about rollers 45 and 47 a number of times to eliminate any possibility of slippage of the yarn thereon. Between draw-off roller 32 and guide roller 43, the yarn is subjected to treatment with a stretching liquid 42, passed on to the yarn by means of conduit 40. The stretching liquid will be described with particularity hereinafter. The draw-off roller and stretching roller are positively driven to impart a portion of the tension and stretch on the yarn between the guide 16 and the roller 30, and a portion between the roller 30 and the roller 45.

The apparatus shown in Figure 3 is particularly useful in such instances where the requisite tension and stretch cannot be imposed on the filaments solely in their travel through the spinning bath. It has been found that when such filaments are passed into contact with a stretching bath, the requisite tension and stretch can be imposed on the yarn during the spinning thereof.

Figure 4 of the drawings discloses a typical gel swelling factor curve for a viscose of a given composition. From this curve, it will be noted that when the acidity of the bath in percentage by weight of sulfuric acid is 12%, the gel swelling factor of the yarn will be slightly under 9.0. When the acidity of the bath is reduced to 11%, the gel swelling factor lies between 5.0 and 6.0. When the acidity is further reduced to 10%, the gel swelling factor drops to between 3.0 and 4.0. With an acidity between 8% and 9%, the gel swelling factor has dropped to a minimum value of 3.0. Further reduction in the acidity of the coagulating bath will cause the gel swelling factor of the yarn to rise again in accordance with the contour of the curve shown in the drawing.

In its broad scope, the process of the present invention is operative and useful with any balanced viscose-sulfuric acid-salt spinning bath system. Particularly desirable crimped yarns and filaments will be obtained in accordance with the following specific combination of relationship factors:

(1) The viscose composition contains between 5% and 100% protein, based on the weight of cellulose content of the viscose.

(2) The viscose-protein composition has an alkali content of between 2% and 7%.

(3) The viscose-protein composition has a salt index of between 1.5 and 6.

(4) The coagulating and regenerating bath has a sulfuric acid content between 60% and 90% of that amount required to produce a yarn having a minimum gel swelling value.

(5) The coagulating and regenerating bath contains between 15% and 30% sodium sulfate.

(6) The coagulating and regenerating bath contains between 0.5% and 3% zinc sulfate.

(7) The temperature of the coagulating and regenerating bath is between 40° C. and 75° C.

(8) The temperature of the relaxing bath is sufficiently high to impart a shrinking action to the filaments at least equal to that of water at 20° C.

(9) Imposing on the filaments, during the spinning thereof, a tension of at least 0.5 gram per denier and a stretch of at least 40%, and after substantially complete regeneration of the

filaments, relaxing the same completely free of all tension in a liquid which will swell the same.

(10) The filaments travel a total length of at least 25 inches in the regenerating and coagulating bath.

In addition to the above mentioned ingredients of the coagulating bath, it is permissible to have present as much as 6% or 7% glucose or similar organic substances well known in the art. The presence of glucose in the spinning bath is not an essential feature of this process, but may be desirable, particularly when continuous filament yarn is produced. As a guide to the proportion of glucose to be used, it may be said that 2% of glucose can replace approximately 1% of sodium sulfate.

In accordance with the above detailed process, the specific enumerated factors are all interdependent and must be adjusted in relation to one another in order to obtain the desired result, i. e. a satisfactory crimp.

It is, of course, understood that relaxing of the filaments in an aqueous medium completely free of all tension is absolutely essential, no matter what variations may be introduced in the other conditions. It is also essential that the tension on the filaments during the spinning (including stretching) be at least 0.5 gram per denier, and that a stretch of at least 40% be placed on the filaments. For each of the factors enumerated above, the range within which the process may be successfully operated has been indicated, but it will be apparent at once to one skilled in the art that if any one of the factors is set at or near the extreme lower or upper limit of its particular range, other factors may have to be adjusted in order to obtain the best results. To illustrate, if the acid content of the coagulating bath is near the lowest limit of the range, it is desirable to adjust some of the other factors to restore the balance of the conditions, for example the zinc sulfate and sodium sulfate contents of the bath. Likewise, the bath temperature should desirably be raised.

In the case of a change in the alkali content of the viscose, I have found that the most important other variable requiring adjustment is the acid content of the coagulating and regenerating bath. As already stated, the acid content necessary to produce a good crimp should be between 60% and 90% of the minimum gel swelling acidity. I have found as an empirical rule that, over the operable ranges shown, a 1% increase in alkali content of the viscose is approximately compensated for by a 1½% increase in the acid content of the coagulating and regenerating bath.

As above stated, it is essential in accordance with this invention that a tension of at least 0.5 gram per denier and a stretch of at least 40% be imposed on the filaments during the spinning thereof. The tension and stretch imposed on the filaments may, of course, greatly exceed that above specified. Any tension or stretch under that which will break the filaments may be used in accordance with the present invention. This tension and stretch must be imposed on the filaments during the coagulation and regeneration thereof when operating without a stretching bath as shown diagrammatically in Figure 1 of the drawings. In some instances, however, it may be impossible to impose that amount of stretch and tension without the use of a stretching bath. Under such circumstances, an arrangement as shown in Figure 3 of the drawings may be used.

In the latter case, the requisite stretch and tension are partially imposed on the filaments during the coagulation and regeneration thereof and partially imposed thereon during the stretching thereof.

The path of the filaments through the coagulating and regenerating bath liquor must be sufficiently long (at least 25 inches and preferably at least 50 inches) to substantially complete the regeneration thereof while in said bath. However, if the stretching bath is capable of regeneration due to heat or content of acid, the regeneration of the filaments may be completed in this bath. For the purposes of the present specification and claims, the spinning of the filaments shall include the passage of the filaments through the stretching bath if a stretching bath is employed.

When a stretching bath is used in accordance with the present invention, it must follow the coagulating bath and the yarn must be passed through the same with a continuation of tension and stretching begun in the coagulating bath. The degree to which the filaments are stretched or tensioned in the coagulating bath may be approximately the same as the degree to which they are stretched or tensioned in the stretching bath. Under some circumstances, it may be desirable to stretch and tension the filaments to a greater degree in the coagulating bath than in the stretching bath. Under other circumstances, it may be desirable to impose a greater degree of stretch and tension on the filaments in the stretching bath than in the coagulating bath. The stretching bath should preferably have a temperature of between about 50° C. and the boiling point thereof. The stretching bath should be composed of a non-alkaline, aqueous liquid preferably containing not to exceed that acidity equivalent to 3% of sulfuric acid. This bath is preferably composed of water.

The relaxing bath may be composed of any liquid which is capable of swelling the cellulose-protein filaments. Since the filaments will be substantially regenerated by the time they are subjected to relaxation in the relaxing bath, the latter will have substantially no regenerating action on the filaments. The relaxing bath preferably comprises water and it may be acidic, neutral, or slightly alkaline. The relaxing bath may contain an acid or a salt such as calcium chloride, sodium thiocyanate, calcium thiocyanate or the like. Such salts will often impart a particularly desirable swelling action to the filaments, whereby crimping takes place in a particularly desirable manner. Such relaxing baths may also contain purification agents such as sodium carbonate, caustic soda and the like, which may, similarly to the above mentioned salts, also have a desirable swelling action on the filaments, but the concentration of such alkaline agents should be low (not over 0.5%) because stronger alkaline solutions may have detrimental effects on the strength of cellulose-protein fibers. The temperature of the relaxing bath may vary widely as this is not critical. The relaxing bath may comprise or consist of organic liquids such as glycerol if the latter is used at a temperature of the order of 120° C., at which temperature glycerol is found to swell regenerated cellulose filaments. Regenerated cellulose-protein filaments may be relaxed in a bath consisting of anhydrous liquid ammonia since the latter is capable of swelling cellulose. The relaxing bath may contain a hardening agent for the protein, for example formal-

dehyde. Whatever the composition and temperature of the relaxing bath may be, the filaments must be allowed to rest in the relaxing bath free of all tension. The filaments may be passed directly to the relaxing bath from the stretching bath in the form of continuous filaments or staple fibers. Alternatively, the filaments passing from the stretching bath may be collected in any desired manner, for example on a bobbin in accordance with the bobbin spinning process, in a bucket cake in accordance with the bucket spinning process, or loosely in a container therefor. The product may be washed acid free, desulfured and/or bleached prior to the time it is immersed in the relaxing bath or it may be relaxed while in the acid state and then washed, desulfured and/or bleached after crimping has been accomplished.

As above set forth, it is essential that the filaments be completely relaxed so that they are free to shrink to the maximum extent. Probably the best method of securing such complete relaxation is to immerse the skeins or staple in the relaxing bath, making sure that there is ample room for the fibers to crimp freely and shrink. If the filaments are not free from all tension, as for example when they are allowed to relax only partially in a wash and bleach machine by hanging skeins on a rod under the weight of a large amount of liquid, the results are found to be unsatisfactory. This time of immersion of the filaments in the relaxing bath is not critical. Under the proper conditions of relaxation, the crimp will be formed in the fibers in the relaxing bath practically instantaneously. It was considered unexpected and surprising that yarns spun under the above described conditions would develop crimp on relaxing in a swelling medium after the yarn had been subjected to washing treatments and other purification treatments, and even after the yarn had been dried prior to relaxation.

The following examples disclose the use of casein and soy bean protein. However, it is possible to use any alkali soluble protein in accordance with the present invention. For example, crimped yarns have been prepared from viscose modified with 5% (based on the weight of the cellulose) of a reduced and regenerated wool obtained by treating natural wool with thioglycolic acid to break down the disulfide linkages, dissolving in alkali and reprecipitating with acid. Among other proteins which may be used may be mentioned albumin, leucosin, the globulins, zein, gliadin, etc. The amount of protein material added to the viscose may vary between 5% and 100% of the weight of the cellulose in the viscose. It is not necessary that the viscose be made first and later modified with the protein since it is possible to add the protein to the cellulose xanthate at the time the viscose dispersion is initially prepared. However, due to the degradative effects of alkali on proteins, it is generally more satisfactory to dissolve the protein in a previously prepared viscose and, thereafter, to spin the resulting mixture as soon as possible. The most efficient method for dissolving a protein, for example casein, in viscose, is to first moisten the protein with water or an aqueous alkaline solution, allow the protein to swell and then to add the swollen protein to the viscose. Under these conditions, the protein dissolves readily in the viscose and only a few minutes stirring are required to obtain a smooth, even dispersion.

The following examples which are not to be considered limitative of the present invention,

illustrate in detail specific steps by which the present invention may be carried out.

#### Example I

Viscose containing 7% cellulose and 6% of total alkali is modified by adding to it a solution containing 7% casein and 6% alkali, the addition being made in such proportion as to produce a spinning dope containing 0.1 as much casein as cellulose. This mixed solution is aged or ripened in the same manner as standard viscose until it has a salt index of 3.9 and is then extruded through a multiple hole (40—0.0035") spinneret into an acid-salt coagulating and regenerating bath containing 8.5% H<sub>2</sub>SO<sub>4</sub>, 19% Na<sub>2</sub>SO<sub>4</sub>, 4% glucose and 0.85% ZnSO<sub>4</sub>. The thread formed is carried around a series of floating guides located in the bath to impart tension thereto and is then taken up on a bobbin rotating at a peripheral speed of approximately 3,500 inches per minute. The total travel of the filaments is approximately 180" and the maximum tension on the thread at the point where it is wound up on the bobbin is approximately 80 grams or 0.53 gram per denier thread. The gel yarn, after collection on the bobbin, is washed free of acid and dried under tension on the bobbin. To produce crimped fibers, it is only necessary then to form the straight thread into skeins and to suspend the skeins free from tension in a bath of hot water (at least 60° C.) or hot dilute (0.3%) solution of sodium carbonate. Crimped fibers obtained in this manner after drying have a wool-like appearance and hand, and if the crimps are removed by stretching, they can be restored by again suspending the skein in hot water free from tension. These fibers can be dyed alone or in mixture with wool using acid or wool type dyes. They also may be dyed with direct or cotton dyes.

#### Example II

Viscose modified by the addition of 15% casein (based on the weight of the cellulose in the viscose) in a manner similar to that described in Example I is spun at a salt index of 4.4 into a bath containing 9% H<sub>2</sub>SO<sub>4</sub>, 23% Na<sub>2</sub>SO<sub>4</sub>, 4% glucose and 0.85% ZnSO<sub>4</sub>. The general procedure used in spinning is the same as that of Example I, except that the final tension in this case is 0.7 gram per denier on the gel filaments. After spinning, the yarn is washed and cut into staples approximately 2 inches in length and the staples are suspended free from tension in a bath of hot water having a temperature of 80° C. On entering the bath of hot water, these filaments crimp strongly and the crimps so produced are relatively permanent in the sense that, if removed by stretching, they may be restored by again immersing the fibers, free from tension, in water having a temperature of 60° C. These fibers, like those of Example I, may be dyed with either wool or cotton dyes and may be used either alone or for blending purposes with a wide variety of other staple fibers.

#### Example III

Viscose containing 7% cellulose and 6% alkali is modified by the addition of sufficient soy bean protein to equal 10% of the weight of the cellulose. The mixed solution is spun under a tension of approximately 0.55 gram per denier using a bath travel of 180 inches and spinning bath similar in composition to that described in Example I. The gel yarn on the bobbin is washed free from acid and is kept for approximately 16 hours

in a 1% solution of formaldehyde to harden or insolubilize the protein. The thread is then relaxed in a bath of water having a temperature of 80° C. with the production of highly crimped fibers which are wool-like in hand and may be dyed with acid or wool dyes.

*Example IV*

Viscose having a normal composition of 7% cellulose and 6% alkali is modified by the addition of an amount of casein equivalent to the cellulose contained in the original solution. To make this addition, 105 parts of casein are moistened with 495 parts of water and, after being allowed to stand for a few minutes to permit thorough wetting of the casein, there are added to it 1,500 parts of viscose. The mixture is then stirred until a smooth uniform dispersion is obtained. The composition of this mixture is approximately 5% cellulose, 5% casein and 4.3% total alkali. The mixed solution is extruded through a multiple hole spinneret into an acid-salt bath containing 5.35% H<sub>2</sub>SO<sub>4</sub>, 23% Na<sub>2</sub>SO<sub>4</sub>, 4% glucose and 0.85% ZnSO<sub>4</sub>. The bath travel is 180 inches and the maximum tension on the thread is approximately 60 grams for 150 denier thread. The acid wet thread collected on the bobbin is cut to staple lengths and, in the absence of any tension, these are suspended in a protein hardening bath comprising 7.6% sodium chloride, 3.9% aluminum sulfate, and 3.3% formaldehyde. A special feature of this process is that the hardening bath serves the dual purpose of a relaxing bath producing crimps in the fibers at the same time that these fibers are toughened and rendered insoluble. The time required for completing the hardening treatment is about 24 hours after which the product is washed, treated with a finish and dried. The resulting fibers are wool-like and dye deeply with most types of wool dyes. They also possess a pleasant, soft hand.

*Example V*

Viscose containing 7% cellulose and 6% alkali is modified by the addition of an amount of casein equivalent to the cellulose content of the viscose, the casein in this case being added in the form of a solution in alkali. The mixed solution then contains 5% cellulose, 5% casein and 6% alkali. In addition, there is added to the solution 0.25% of a styrene/maleic anhydride interpolymer which has the property of functioning as a protein hardening agent. The bath composition used for spinning contains 8.1% H<sub>2</sub>SO<sub>4</sub>, 23% Na<sub>2</sub>SO<sub>4</sub>, 4% glucose and 0.85% ZnSO<sub>4</sub>. The spinneret used contains 60 holes of 0.0035" diameter each. The bath travel is 120", the bath temperature 55° C., the thread speed at the bobbin 3500"/min. and the tension on the thread at the bobbin approximately 0.4 g/d. After spinning the thread is cut into staples and relaxed completely in water having a temperature of 70° C. The resulting fibers are highly crimped and the crimps are permanent in the sense that, if temporarily removed by stretching they may again be recovered by suspending the fibers in a liquid swelling bath free from tension.

*Example VI*

Viscose, 7% cellulose and 6% alkali, is modified by the addition of 33% casein and 2.5% of a styrene/maleic anhydride interpolymer (both based on the cellulose contained in the viscose). Sufficient alkali is also added to maintain the original alkalinity of the viscose and the resultant

spinning solution which contains 6% cellulose, 2% casein, 0.25% styrene/maleic anhydride interpolymer and 6% total alkali is spun into filaments in a manner similar to that described in Example V except that the bath used contains 7% sulfuric acid, 23% Na<sub>2</sub>SO<sub>4</sub>, 4% glucose and 0.85% ZnSO<sub>4</sub>. Maximum tension on the thread at the bobbin in this case is approximately 0.6 g/d. and after spinning the gel thread is cut into staple lengths without intermediate washings and the staples are permitted to relax completely in hot (80-90° C.) water. The staples obtained are finely crimped, can be dyed with acid dyes and have a pleasant wool-like hand.

The crimped filaments and fibers produced by the process of the present invention are entirely new and different in character from any previously known crimped regenerated cellulose-protein filaments or fibers. They are characterized by unique and outstanding properties not found in the crimped fibers produced heretofore. One of these entirely new and unexpected properties lies in the fact that the crimp, after being removed through stretching, combing, or other mechanical treatment, is substantially completely restored to the fiber simply by suspending it in water, or other aqueous liquid, in the absence of tension. The crimp regain is practically instantaneous, whether the fiber treated be in the form of staple or of continuous filaments. It can be readily demonstrated by manually stretching, or repeatedly combing a sample of crimped fiber so as to destroy its crimp, then immersing the sample in water, whereupon it at once crinkles and crimps to give the original structure. This surprising property is, of course, of great importance in the industrial processes to which the fibers may be subjected. For example, carding usually destroys, at least partly, the crimp in an ordinary crimped fiber. Fibers made by this process, however, may be carded and afterward immersed in water, whereby the original crimp is restored completely or substantially so. No previously known crimped regenerated cellulose-protein fibers even remotely possess this remarkable characteristic.

It is theorized that the production of crimped high tenacity fibers according to this invention is possible primarily by reason of the fact that during spinning there is formed in individual filaments a certain kind of non-uniformity with respect to the orientation of the cellulose comprising the edges or outside boundary of the filament as compared with that comprising the interior sections of the filament. When fibers possessing such non-uniformity in their cross sections are permitted to shrink freely, the different layers of regenerated cellulose do not shrink to the same extent and the fibers tend spontaneously to fold over and produce a crimped effect. For this reason, use is made of the high spinning tensions which are a fundamental feature of the present invention. A proper balance between the above described relationship factors is considered to be essential since only under such selected conditions is the rate of penetration of acid into the thread such that a good differentiation can be obtained between the degree of orientation of fiber wall and fiber core. There is a possibility that differences in the fiber structure (density and degree of orientation) occur across the filament which ultimately cause the fiber to crimp when relaxed. The foregoing theoretical discussion is not, however, to be construed as limiting the process of this invention.

The high tenacity crimped fibers which may be obtained as a result of the present invention are characterized by filament strength of from 2.25 to over 3 grams per denier dry tenacity, and from 1.25 to over 2 grams per denier wet tenacity. The dry extensibilities, after straightening the crimp therefrom, for threads formed in accordance with the present invention are of the order of 10% to 20%, depending on the spinning tension used in their formation, and in general, it can be said that the extensibilities of crimped fibers produced in accordance with the present invention are better than those of straight fibers of equal tensile strength but spun without permitting free shrinkage. The curly crimp in the fibers produced in accordance with the present invention is durable and produces a pleasing, wool-like appearance and hand. In the case of fibers which have been cut to staple length before being permitted to relax in water, the crimps obtained are quite irregular, both as to their number per inch and their arrangement around the fiber axis. It is difficult, therefore, to define the degree of crimp obtained in these fibers in a quantitative manner, but in general, it may be said that the number of crimps per unit length along the axis of the unstretched fiber is above 10 crimps per inch. This means that these fibers are easily distinguishable from ordinary regenerated cellulose staple fibers, or any previously known regenerated cellulose-protein fibers, even those made by the so-called "acid-cutting" process, since at most the latter do not show more than 5 or 6 crimps per inch. The crimps in the fibers are remarkably resistant to laundering with soap. As has been mentioned previously, even after removing the crimp by stretching the filaments, the crimp can be restored by subjecting the filaments or fibers to another relaxing treatment in a liquid.

Continuous filament yarn comprising crimped filaments of the type hereinabove described is particularly desirable for the production of woven and knit goods where more than average yarn strength, together with a wool-like hand, is desired. The crimped staple fibers of the present invention are very desirable for the production of a unique and superior spun yarn. Fabrics produced from both continuous filament and spun yarn made in accordance with the present invention will have a very desirable hand, due to regain of filament and fiber crimp upon wetting.

Since it is obvious that many changes and modifications can be made in the above described details without departing from the nature and spirit of the invention, it is to be understood that the invention is not to be limited to the said details except as set forth in the appended claims.

I claim:

1. A process for the production of crimped regenerated cellulose-protein filaments and fibers which comprises the steps of spinning filaments from a viscose solution containing from 5% to 100% protein, based on the weight of the cellulose in the viscose, into a coagulating and regenerating bath and then, after regeneration is substantially complete, relaxing the same completely free from all tension in a liquid which will swell the same, said steps being carried out in accordance with the following relationship factors: (1) The viscose-protein composition has an alkali content of between 2% and 7%; (2) The viscose-protein composition has a salt index of

between 1.5 and 6; (3) The coagulating and regenerating bath has a sulfuric acid content between about 5.35% and 9.00% and between 60% and 90% of the minimum gel swelling factor acidity; (4) The coagulating and regenerating bath contains between 15% and 30% sodium sulfate; (5) The coagulating and regenerating bath contains between 0.5% and 3% zinc sulfate; (6) The temperature of the coagulating and regenerating bath is between 40° C. and 75° C.; (7) The temperature of the relaxing bath is sufficiently high to impart a shrinking action to the filaments at least equal to that of water at 20° C.; (8) Imposing on the filaments during the spinning thereof a tension of at least 0.5 gram per denier and a stretch of at least 40%; (9) The filaments travel a total length of at least 25 inches in the regenerating and coagulating bath.

2. A process as defined in claim 1 in which said filaments are passed, in the spinning thereof, through a non-alkaline stretching bath containing not to exceed that acidity equivalent to 3% sulfuric acid.

3. A process as defined in claim 1 in which said filaments are passed, in the spinning thereof, through a non-alkaline stretching bath containing not to exceed that acidity equivalent to 3% sulfuric acid and having a temperature between 50° C. and the boiling point thereof.

4. A process as defined in claim 1 in which said filaments are passed, in the spinning thereof, through a stretching bath composed essentially of water having a temperature between 50° C. and the boiling point thereof.

5. A process as defined in claim 1 in which said filaments are passed, in the spinning thereof, through a non-alkaline stretching bath containing not to exceed that acidity equivalent to 3% sulfuric acid and in which at least a portion of said tension and stretch is imposed on the filaments in the spinning bath and a portion of said tension and stretch is imposed on the filaments in the stretching bath.

6. A process as defined in claim 1 in which said relaxing liquid is water.

7. A process as defined in claim 1 in which said filaments are passed, in the spinning thereof, through a non-alkaline stretching bath containing not to exceed that acidity equivalent to 3% sulfuric acid and in which said relaxing liquid is water.

8. A process as defined in claim 1 in which said filaments are passed, in the spinning thereof, through a non-alkaline stretching bath containing not to exceed that acidity equivalent to 3% sulfuric acid and having a temperature between 50° C. and the boiling point thereof and in which said relaxing liquid is water.

9. A process as defined in claim 1 in which said filaments are passed, in the spinning thereof, through a stretching bath composed essentially of water having a temperature between 50° C. and the boiling point thereof and in which said relaxing liquid is water.

10. A process as defined in claim 1 in which said filaments are passed, in the spinning thereof, through a non-alkaline stretching bath containing not to exceed that acidity equivalent to 3% sulfuric acid and in which at least a portion of said tension and stretch is imposed on the filaments in the spinning bath and a portion of said tension and stretch is imposed on the filaments in the stretching bath and in which said relaxing liquid is water.

11. A process as defined in claim 1 in which

the filaments are relaxed in the relaxing bath immediately after stretching the same.

12. A process as defined in claim 1 in which the filaments are collected on a yarn support and subjected to a washing treatment after stretching and prior to relaxing.

13. A process as defined in claim 1 in which the filaments are collected on a yarn support and subjected to a washing and drying treatment after stretching and prior to relaxing.

14. A process for the production of crimped regenerated cellulose-protein filaments and fibers which comprises the steps of spinning filaments from a viscose solution containing from 5% to 100% protein, based on the weight of the cellulose in the viscose, into a coagulating and regenerating bath and then, after regeneration is substantially complete, freely suspending the filaments in filamentous structure form in an aqueous liquid bath having a strong shrinking action on the filaments and in complete absence of tension, to completely relax the same, said steps being carried out in accordance with the following relationship factors: (1) The viscose-protein composition has an alkali content of between 2% and 7%; (2) The viscose-protein composition has a salt index of between 1.5 and 6; (3) The coagulating and regenerating bath has a sulfuric acid content between 5.35% and 9.00% and between 60% and 90% of the minimum gel swelling factor acidity; (4) The coagulating and regenerating bath contains between 15% and 30% sodium sulfate; (5) The

coagulating and regenerating bath contains between 0.5% and 3% zinc sulfate; (6) The temperature of the coagulating and regenerating bath is between 40° C. and 75° C.; (7) The temperature of the relaxing bath is sufficiently high to impart a shrinking action to the filaments at least equal to that of water at 20° C.; (8) Imposing on the filaments during the spinning thereof a tension of at least 0.5 gram per denier and a stretch of at least 40%; (9) The filaments travel a total length of at least 25 inches in the regenerating and coagulating bath.

15. A process as defined in claim 14 in which the relaxing treatment liquid is water having a temperature of at least 20° C.

16. A process as defined in claim 14 in which the filaments are stretched in a secondary bath comprising water having a temperature of at least 60° C.

17. A process as defined in claim 14 in which the filaments are subjected to a washing treatment after regeneration and prior to said relaxing treatment.

18. A process as defined in claim 14 in which the filaments are subjected to a washing treatment and dried after regeneration and prior to said relaxing treatment.

19. A process as defined in claim 14 in which the relaxing bath comprises a dilute solution of formaldehyde.

WILLIAM D. NICOLL.

No references cited.

Patent No. 2,515,889

**Certificate of Correction**

July 18, 1950

WILLIAM D. NICOLL

It is hereby certified that error appears in the printed specification of the above numbered patent requiring correction as follows:

Column 8, line 25, before the word "thread" insert *for 150 denier*; column 10, line 32, for "somples" read *sample*; column 14, line 28, for the claim number "18" read *19*;

and that the said Letters Patent should be read as corrected above, so that the same may conform to the record of the case in the Patent Office.

Signed and sealed this 17th day of October, A. D. 1950.

[~~seal~~]

THOMAS F. MURPHY,  
*Assistant Commissioner of Patents.*